

Oct. 26, 1965

R. M. BRICK ET AL  
PREPARATION OF LAMINATE METAL STOCK BY  
USE OF ORGANIC ANTI-WELDING MATERIALS  
Filed July 20, 1960

3,214,251

FIG.1



FIG.2



FIG.3



FIG.7



FIG.4



FIG.8



FIG.9



FIG.6



INVENTORS  
ROBERT M. BRICK,  
ROBERT B. MESROBIAN  
& ANTS HANSSON

Macmillan, Parker, Dillon & Stewart,

ATTORNEYS

1

3,214,251

**PREPARATION OF LAMINATE METAL STOCK  
BY USE OF ORGANIC ANTI-WELDING  
MATERIALS**

Robert M. Brick and Robert B. Mesrobian, Hinsdale, and  
Ants Hansson, Evanston, Ill., assignors to Continental  
Can Company, Inc., New York, N.Y., a corporation of  
New York

Filed July 20, 1960, Ser. No. 44,148  
28 Claims. (Cl. 29—183)

This invention relates to the employment of organic materials for preventing the welding of metal in the making of laminate stock.

It is known to provide a metal billet with an internal discontinuity containing an anti-welding or resist material, and to roll the same for producing a laminate stock. Prior practices have been to employ refractory solid powders such as alumina, silica, mica, talc, gypsum and the like, for the reason that the rolling is most, efficaciously effected by a schedule of heat treatments, with successive hot and cold rolling. The billet could be an ingot having one or more longitudinal channels filled by such a resist, and produced by casting the metal around a coherent core of such resist material; or longitudinal hollow channels could be formed during casting, or subsequently by drilling, and later filled with the resist material. The billet may be originally 8, 12 or more inches in thickness, and the internal discontinuity may be  $\frac{1}{2}$  inch or more thick; noting that when the refractory resist powder is later introduced, the permissible minimum thickness depends upon the ability to produce an essentially uniform deposit of the powder therein; and that when a preformed core of coherent refractory powder is used, a similar minimum must be observed to avoid disruption during the casting. The purpose of the resist or anti-welding compound is to prevent the welding or sticking together of the laminations, and for this a microscopically thin film is as effective as a thicker one: noting that the metal provides the laminations which produce the final product. It is desirable to keep the resist dimension as thin as possible in the ingot but thicknesses of less than a half-inch, in an ingot which is 6 to 14 feet long, are not easily filled to uniform packing density with a dry refractory powder.

When a refractory powder is employed as the resist, and the rolling operation produces a relative displacement of the powder along the internal discontinuity during the rolling, a part of the powder is usually expelled at the trailing end as this passes through the rolls. Refractory powders such as aluminum oxide are frequently employed, which are recognized abrasive agents; and the expelled powders can damage the rolls and their bearings.

Most organic materials undergo extensive thermal decomposition upon heating in air at temperatures around 500 degrees F. Such decomposition may be by any of a group of complex reaction including depolymerization or disproportionation; and particularly may be catalyzed by contact with metal. In general, it has been expected in the art of coating with organic enamels or lacquers that breakdowns will occur at temperatures of 600 degrees F. or below even with very short exposure time. On the other hand, normal heat treatment and hot rolling schedules for aluminum, copper, zinc, magnesium and other non-ferrous metals and their alloys call for heating to a temperature of around 445 to 540 degrees C. (700 to 1,000 degrees F.) for periods of ten minutes up to four or more hours.

It has now been found that liquefiable materials as set out hereinafter may be introduced into billet channels, with the billet being heated and then subjected to a

2

schedule of hot and cold rolling, without loss of the ability of the organic compound to function as an anti-welding material during the hot and cold rolling operations by which a billet 12 inches thick may be reduced to a total thickness of, say, 0.016 inch with two metal laminations each 0.008 inch thick being separated by a microscopically thin residual layer of the resist material. The function of preventing welding is then not dependent upon the particle size of the resist residue, and therewith the original channel in the billet, for receiving the resist, may be made much thinner than with powder resists, e.g., organic resists in channel  $\frac{1}{8}$  inch or less thick are found as effective in an ingot as a powder resist thickness of  $\frac{1}{2}$  inch or more, and therewith caliperings of the final thickness of the rolled laminate strip can directly determine the thickness of each lamination without need of allowance for the resist residue.

Hot rolling, as applied to the metal, herein refers to a temperature condition at which the metal does not exhibit strain-hardening; and cold-rolling of the metal to a temperature at which strain-hardening occurs. For example, hot-rolling of aluminum alloys ceases as the material cools to about 650 degrees F., and the subsequent rolling at lower temperatures effects strain-hardening.

Further, organic compounds can be chosen, in accordance with this invention, which do not require removal, but which bond directly with later-applied organic enamels and lacquers and in effect become a part thereof.

The word "liquid" is herein used to define that state of the selected anti-welding substance in which the molecules are able to change their positions plastically with respect to one another at the temperature and under the local pressure effects of hot-reduction of the metal which surrounds and encloses the substance and in which the said substance spreads to occupy the cross-section of the channel during the hot-reduction: with the relative movement being restricted by inter-molecular forces so that an essentially fixed volume is maintained. Therewith the substance does not fracture under the heat and pressure of hot reduction, but retains continuity and in part moves along the channel as the metal and the anti-welding substance are being reduced in thickness and extended in length. The word "solid" is herein used to define that state at a lower temperature of an organic compound, which is liquid at a higher temperature, at which the molecules are so strongly coupled that the compound does not flow under the action of gravity, and in which it exerts a stiff resistance to molecular change of relative position but has capability of being extended and of maintaining a continuous layer between the surfaces of the channel during cold-reduction, without exhibiting brittleness or breaking into fragments which separate from one another during the course of the cold reduction and permit the movement of the metal forming such surfaces into welding contact with one another. The words "melting" and "liquefaction" are used herein to define the change of such anti-welding substances, upon heating to the hot reduction or treating temperature, so that its viscosity is lowered and its ability to flow is increased whereby it spreads and produces within the billet being rolled a continuous body of weld-preventing material.

An object of this invention is the preparation of a metal billet containing a longitudinal internal channel, and the heating and rolling of the same for producing a laminate strip, with the employment in the channel of an anti-welding or resist material which is stiffly resistant to flow at room temperature, which becomes liquid at the temperature and pressure scheduled for the hot-rolling of the billet, and which is later effective during cold-rolling to undergo deformation and extension or for maintaining its anti-welding action.

Another object of this invention is the preparation of a metal billet containing an organic resist, and the reduction of the same to a desired over-all thickness by a schedule including hot-rolling and heat treatment at temperatures appropriate to the metal.

Another object is the employment, as a resist, of a material of non-abrasive characteristics, and therewith having essentially no abrasive action upon the rolls, tools, and other equipment coming in contact therewith.

Another object is the employment, as a resist, of an organic compound compatible with an organic enamel or lacquer later applied therover.

A further object is the employment, as a resist, of an organic compound which, during the course of a schedule of hot and cold rollings, remains effective to prevent welding of metal laminae separated thereby, and to maintain such behavior in extremely thin layers and therewith provide smooth adjacent surfaces on such laminae.

A further object is the preparation of laminate stock by forming an ingot with a small internal channel, filling the channel with a resist which is liquid at the beginning of hot-rolling, and final rolling of the same with passes which are at temperatures under which the resist is essentially an extensible solid.

With these and other objects and features in view, as will appear in the course of the following description and claims, illustrative embodiments of the invention are set out in conjunction with the accompanying drawings, in which:

FIGURE 1 is a perspective view of part of a billet having core channels or internal discontinuities with parallel plane sides and chisel-shaped edges;

FIGURE 2 is a perspective view of a part of a billet having core channels of rounded edge form;

FIGURE 3 is a perspective view, showing the ingot end being closed by peening and welding;

FIGURE 4 is a perspective view of an ingot having longitudinal internal channels, being filled with an organic resist;

FIGURE 5 shows in conventionalized block form a schedule of heating and rolling operations;

FIGURE 6 is a conventionalized perspective view showing the placing of a resist in a billet channel immediately prior to hot rolling;

FIGURE 7 shows, on a larger scale than FIGURES 1 to 6, a part of a multi-wide rolled strip;

FIGURE 8 shows the opening or expansion of a section of the strip to form a tubular body;

FIGURE 9 shows the application of an organic enamel to the interior surface of such a body.

It has been found that many high molecular organic compounds can be employed as anti-welding or resist materials in hot working billets into laminate stock, e.g., with a schedule of heatings and hot rollings, when they are protected from oxygen during the operations. Such can be accomplished by heating the billet to hot-rolling temperature, introducing the resist into the internal channel or channels, then performing a first rolling step for distributing the resist and reducing the channel sections so that the same are filled with resist essentially from end to end of the billet, whereby the billet itself prevents access of air to the resist except at the end openings of the channels, and continuing the hot rolling prior to the cooling of the billet and within a time period of a few minutes: noting that many of the compounds degrade at a time-temperature function which enables them to remain effective as resists for times up to an hour or more and that all named compounds remain effective for at least five minutes at the hot-rolling temperatures provided that the air exposure prior to completion of the first pass is restricted. Alternatively, the protection from oxygen can be accomplished by placing the resist in such discontinuities and sealing the openings as by welding, before subjection to the high heating of the specified schedule. The resist may be inserted into the cold billet block, the

block welded, and the scheduled heatings and workings performed; or the block may be heated to a temperature effective for liquefying the resist without its degeneration in the presence of air, filled and then welded shut, and the scheduled heatings and workings performed. In cases

where the resist is charged into a cold billet, or into a billet heated to the temperature for liquefaction but not a quick degradation of the resist when heated in contact with air, a preliminary breakdown or conformance rolling may be accomplished to distribute the resist and reduce the channel section so that it is filled by the resist with expulsion of air, before the billet is heated to the temperature for the start of the hot rolling. The choice of specific procedure depends upon equipment available and economics, and upon the physical form of the resist at room temperature. For example, when the resist is in powdery form, the melting and the escape of air from the pores may cause bubbling with passage of some of the liquid material into regions where closure welding is to be done; and in such cases, a low temperature heating for liquefaction is preferred, followed by the expulsion of air before the closure and heating to hot rolling temperatures. On the other hand, if the available equipment permits the homogenizing heating of the empty billet, followed by a quick introduction of the resist, no sealing of the charged end of the channel is necessary, if this charging is quickly followed by the initiation and completion of the hot rolling.

It has been found that organic resists which appear harder than the billet metal can be employed, in cold rolling, provided that the film is thin relative to the thickness of the metal laminations during the rolling pass. For example, an epoxide resin (e.g., that sold commercially under the name Epon-1007), which appeared harder than aluminum, could be employed successfully by heating the billet and hot rolling until the epoxy resin resist film had a thickness of a few thousandths of an inch, during which the resist spread easily as a film: thereafter, a cold rolling proceeded with extension of the film by rupture into flakes which flattened and spread and prevented cold welding.

In general, these organic resists work both when the rolling is hot with little work-hardening of the metal; and later when the rolling is cold with a relatively high work-hardening of the metal.

A characteristic observed is that, because many of the resist materials appear to have greater adhesion to the metal than cohesion, the final strip produced permits the opening or expansion with both internal metal surfaces having parts of the residual resist layer clinging to them.

Examples of practice in which the empty billet is heated to hot rolling temperature, charged with resist, and quickly rolled, are:

#### Example 1

An aluminum billet having a longitudinal internal channel was welded closed at one end. The billet was heated to 900 degrees F.; the open end raised, and a solid epoxide resin introduced as a resist into the channel until the channel was substantially full. The resin melted as it entered and flowed downward to form the fill. The epoxide resin was a bis-phenol epichlorohydrin condensate, and is illustrative of the epoxy resins which can be employed, being a solid at room temperature and becoming liquid at 300 degrees F., being obtainable as flakes or pellets which may be converted to a powder: the resin commercially available under the trademark Epon-1007 was satisfactory. The billet was immediately hot-rolled, with the open or charging end first presented to the rolls; and then cold-rolled, preferably after an anneal reheating to 900 degrees F., and a cooling before the cold-rolling. An original billet of 2 to 12 inch thickness can be hot-rolled to, say, 0.120 inch thickness, and then reduced to 0.016 inch by cold-rolling, to provide a laminate strip having two metal laminations connected integrally

at the strip edges and separated from one another by the microscopically thin residual layer of the resist material. The laminations can be separated, and opened out or expanded to form a tubular structure: the resist residue, after the opening, was found to have darkened but not charred, being soluble in acetone, with no damage indicated upon infra red examination.

*Example 2*

A red brass billet (85 percent copper, 15 percent zinc) having an internal longitudinal channel with a metal wall thickness of  $\frac{1}{16}$  inch was heated to 950 degrees F., a slab or strip of the epoxide resin of Example 1 was introduced, and the hot rolling immediately started, bringing the billet to 0.060 inch gauge. The strip was annealed at 1,100 degrees F., cooled and cold-rolled to a final gauge of 0.016 inch. The metal laminations could readily be separated and bent apart to form a tubular body. Although there was no visually detectable epoxide residue on the interior, solvent extractions of the surface and infra red analyses indicated the presence of epoxide. The internal surfaces were smooth and had a bright appearance.

*Example 3*

Like operations with billets of aluminum, zinc, magnesium and copper, and their alloys, can be performed with polyethylene as a resist, e.g., the so-called regular branched type sold under the trademark Dynk by Union Carbide Plastics Co., or the linear type sold under the trademark Marlex by Phillips Petroleum Company, or the commercial polyethylenes of other suppliers. These are obtainable in pellets which are solid at room temperature, rubbery at 300 degrees F., and melt easily when heated to 360 degrees F. or above. Such are charged into the heated billet, and the schedule of rolling from 900 degrees F. was accomplished. Upon opening the hot and cold rolled strip, the interior was found in good condition.

In the practice of Examples 1 to 3, it was found that very thin channels were sufficient: and that a large part of the resist could be squeezed out, during the succession of rollings, without the residual film losing ability to prevent welding: that is, the thickness of this film was not apparent to the eye, and probably was of the order of a few ten-thousandths of an inch or less. The resist so expelled, during the early stages of hot-rolling, darkened and charred upon the air exposure, but such charring did not occur internally when the air access was prevented by the surrounding metal.

Examples of practice in which the resist was charged into a warm billet which was then sealed, heated and rolled, are:

*Example 4*

Billets of aluminum, zinc, magnesium, and copper, and their alloys, with an end of each sealed, were heated to 350 degrees F., and charged with pellets of commercial polypropylene (e.g., that available commercially under the trademark Profax), which was solid at room temperature and became rubbery at 300 degrees F. The pellets melted and the resist filled the channel without porosity. The open ends were welded shut without incident. The charged and sealed billets were heated to 900 degrees F. and rolled. After the schedule of hot and cold rolling, the laminations of the strip can be easily separated, and the interior surfaces and residual resist were found in good condition, without welds.

*Example 5*

Billets as in Example 4 were prepared, heated to 360 degrees F., and charged with the polyethylene pellets. The open ends were welded shut, and the billets heated to 900 degrees F. and rolled. There was minor leakage at welds, with darkening of the exudate: but the interiors were in good condition after opening.

*Example 6*

A silicone resin (e.g., that sold under the Dow-Corning trademark Z-6018) can be used as the resist during a heating and hot rolling schedule. A heat-hardening cyclic tetramer resin was used, of the approximate formula



where R is a phenyl and R' is an isopropyl group. This is effective up to temperatures of 900 degrees F. in billets 20 of aluminum and its alloys. Upon filling into the channel with the billet at 300 degrees, the hard solid became liquid with some foaming. The end was welded shut, and the billet heated to 900 degrees F. in its schedule. When there was leakage by imperfect welding, the exudate 25 showed polymerization: the internal resin, after cooling, was found to be a porous hard resin which swelled in acetone but was not totally soluble and exhibited no damage under infra red examination.

The same silicone resin was loaded into a cold ingot, 30 the ends welded shut, and the ingot heated to 900 degrees F. and rolled hot and cold to 0.016 inch thickness. The laminations separated easily, and the internal appearance was of smooth bright metal. The residue was of microscopic thinness but had continued in its weld-preventing 35 behavior.

The practices with the resists of Examples 1 to 3 can be performed by charging the resist into the channel or 40 channels of a cold ingot, sealing as by welding, and then heating to hot rolling temperature and effecting the schedule of rolling operations: and the resists of Examples 4 to 6 can be employed by pre-heating the ingot to hot-rolling temperature, quickly charging with the resist and 45 immediately conducting at least the breakdown or conformance passes of hot-rolling. In general, the channel thicknesses of the ingots or billets are determined by the necessities of making such channels, rather than by the need of having a large quantity of the resist originally present. Therewith, the channels may be open at the ends or become opened by internal liquid pressure during 50 the rolling, so that half or more of the resist escapes without provoking welding, during the course of the hot-rolling. Thus, when a billet has been reduced from 8 inches to 2 inches total thickness, the internal layer of resist may be of the order of one or two thousandths of 55 an inch: and this billet can be further reduced to a strip of 0.250 inch or less thickness without welding, with most of the resists set out.

In general, it has been found that the behavior of the resist during a hot-rolling schedule of up to 15 minutes 60 can be predicted by noting the behavior of the resist when heated for a like time in a sealed autoclave of the metal. Thus, with Example 1, a parallel test by welding the billet at one end, heating to 300 degrees F., charging essentially 65 fully with the epoxy resin pellets and permitting foam to subside, sealing the other end by welding, and then heating to 900 degrees F. for an hour, resulted in some leakage apparently by weld imperfection with the effluent charring, whereas after cooling and opening, the internal protected resist had not charred and infra red examination 70 did not indicate damage.

*Example 7*

An aluminum block having an internal channel was 75 filled at room temperature with a polycarbonate resin,

(e.g., that available commercially under the tradename Lexan, of the formula



where  $n$  represents as usual the number of the stated units in the polymer. The open end is easily welded shut, and no leakage develops during the heating to 900 degrees F. After heating, the resist is found in good condition, as a hard tough resin which is insoluble in acetone, and shows no damage under infra red examination.

An ingot of 3003 aluminum alloy, over 4 inches thick with a core channel about 0.125 inch thickness, was homogenized 18 hours at 1,100 degrees F. and cooled to room temperature. The scalped thickness was 4 inches. The channel had V sections at its edges,  $\frac{1}{2}$  inch wide with a 0.005 inch edge radius. The billet was thoroughly cleaned, and one end welded with a flux coated 1100 welding rod. Polycarbonate pellets were tamped to essentially fill the channel with a packing density of 55 percent. The open end was closed by like welding. The billet was then held for an hour in a furnace at 900 degrees F. Leakage through the welds developed: with carbonaceous deposit in the furnace. The hot billet was then subjected to thirteen hot rolling passes, reducing it from 4 inches to 0.15 inch: it was annealed and rolled to 0.090 inch, followed by a further annealing. It was reduced to 0.024 inch in two passes, again annealed, and rolled to 0.016 inch. Each intermediate annealing was for one hour at 800 degrees F. The rolled strip was completely openable.

*Example 8*

A linear polyamide resin (e.g., one of those polycaprolactams known commercially by the tradenames nylon-6 or Zytel) having the following structure



is employed by introducing the pellets into an aluminum billet while the latter was heated to 440 degrees F., at which temperature the resin is rubbery and can be packed. The closure welding is effected. When, because of imperfect welding, there was minor leakage, there was charring of the exudate during heating for one hour at 900 degrees F. After the heating at 900 degrees F., the internal residual resin material is a light straw-colored cheesy solid, insoluble in methyl alcohol, and showing no damage under infra red examination.

*Example 9*

A hollow aluminum billet with the channel closed at one end was heated to 300 degrees F., and commercial iron stearate introduced and the channel welded shut. This was a mixture of ferric tristearate and  $(St)_2Fe-O-Fe(St)_2$  where St denotes  $\cdot O-CO-(CH_2)_{17}-H$ . It was a dry powder at room temperature and liquid at 300 degrees F. When there was leakage, due to imperfect welding, during heating to 900 degrees F., the exudate charred but the internal material was found not to have changed visually, being insoluble in acetone, and showing no damage under infra red examination.

*Example 10*

The procedure of Example 9 was followed, with aluminum stearate, which is a dry powder at room temperature and is rubbery at 300 degrees F. The billet was heated to 380 degrees F. for the loading; and the billet channel welded shut before heating to 900 degrees F. Again, when, because of imperfect welding, there was leakage, there was charring of the exudate. The internal material yellowed but was otherwise visually unchanged; it was insoluble in acetone and showed minor damage upon infra red examination.

A billet as in Example 7 was first heated at 900 degrees F. for three hours, with one end welded. It was then placed vertically, and the aluminum stearate powder introduced, with melting. The billet was then immediately pushed horizontally into the rolls for the first pass, starting with the open end: and the same rolling and annealing schedule observed. The welded trailing end burst open at the first pass, and much liquid resist was discharged. The rolled strip was completely openable.

The tests of Examples 7 to 10, and like tests with the resist materials and metals of Examples 1 to 6, have been made at temperatures exceeding 900 degrees F. for times up to an hour and a half or more, with the stated results. Such materials thus can be employed in the procedures of Examples 1 to 6, by heating prior to the charging, or by charging at a low temperature and then sealing and heating, and with the performance of hot-rolling operations at like temperatures of 900 degrees F. or over, all within the time during which the resist material remains effective. When lower temperature:time factors are involved, other organic materials may be employed.

*Example 11*

A terephthalic-isophthalic polyester (e.g., that commercially available under the tradename Videne), which is commercially available in pellets which become rubbery at 300 degrees F., was employed. It had the general formula



where R represents the para- or meta-phenyl nucleus singly or in mixture. The hollow aluminum billet was heated to 350 degrees F., loaded, and welded closed. Minor leakage of a resinous material occurred during heating for a hour to 900 degrees F. Upon cooling, the internal resin was a yellow wax-like solid which exhibited the effects of some depolymerization: it was insoluble in acetone or toluene, and had suffered no damage, according to infra red examination. It may be noted that infra red examination can reveal change of intra-molecular structure, but is not a sure guide as to polymerization or partial depolymerization.

*Example 12*

A novolac phenolic resin (e.g., that available under the tradename BR-254, Union Carbide) has been employed under the stated heating to 900 degrees F., with aluminum. The resin was a para-phenylphenol-formaldehyde resin of the formula



being a hard solid at room temperature, and a liquid at 300 degrees F. The resin commercially available under the trademark BR-254 was used. This was charged into the cold billet; the billet was welded shut and heated to 900 degrees F. After cooling and opening, the resin had a very dark color, was partially soluble in acetone, and exhibited no damage effect under infra red examination.

A billet was filled with the phenolic resin at room temperature to a packing density of 85 percent, as described for Example 7, and rolled with like annealings. The rolled strip was completely openable.

A like billet was heated at 900 degrees F. for three hours, with one end welded shut. It was placed with the open end up, and the phenolic resin introduced to sub-

stantial filling; then lowered to horizontal, and a like rolling schedule performed. The welded end burst open during the first rolling pass and a large amount of the liquid resist was discharged. The rolled strip was completely openable.

*Example 13*

A hard, solid, complex cyclic hydrocarbon polymer resin prepared from terpene and known as terpene resin (the commercial material available under the trademark Piccolyte S-135 of the Pennsylvania Industrial Chemical Corporation, was used) was loaded into a hollow aluminum billet heated to 300 degrees F., with some foaming. Upon welding and heating to 900 degrees F., cooling and opening, the residue showed that depolymerization to a liquid had occurred, but infra red examination indicated no damage.

*Example 14*

A polymethyl styrene resin was used, of the general formula



This is commercially available as pellets under the trademark Cynac-400 from the American Cyanamid Company; and is rubbery at 300 degrees F. The billet was heated to 340 degrees F., loaded, and the ends welded shut. Upon heating to 900 degrees F., there was leakage of a resinous material. Upon cooling, the internal resin was an amber-colored, fused, hard, brittle resin; soluble in toluene, but showing no damage under infra red examination.

Polystyrene resin was packed to 50 percent density into a billet at room temperature, as set out for Example 7: the billet was then welded closed, and subjected to the heating and rolling schedule as in Example 7. The rolled strip was completely openable.

The materials of Examples 11 to 14 can be employed as in Examples 1 to 6.

*Example 15*

A magnesium billet had its internal channel filled with epoxide resin, as in Example 2, and sealed. It was heated to 700 degrees F. and hot rolled. The internal surfaces were smooth and bright.

The surface effect produced by the use of resists which are liquid during at least the early part of the hot rolling may be illustrated by:

*Example 16*

An aluminum billet 2 inches thick, with a 0.100 inch thick channel, received a polyethylene strip about 0.005 inch thick and slightly narrower than the channel width, at room temperature. It was welded shut and heated to 600 degrees F., and warm-rolled to 0.016 inch in the range 600 to 300 degrees F. During the early passes, the liquid resist broke the weld at the trailing end of the billet and a part of the resist was squeezed out. Upon opening, the internal surface was exceptionally bright, indicating that the material was liquid or highly plastic during the rolling. Both internal surfaces had resist material adherent thereto, as shown by the lesser action of caustic solutions than at exterior surfaces or file-cleaned surfaces.

The protective effect of the metal during the hot stage is brought out by the instances where leakage past a weld occurred; noting that the exudate darkened and decomposed under like temperature condition whereas the encapsulated resist exhibited its desired properties.

Practice with the foregoing materials is shown in the drawings. In FIGURE 1, the ingot B has internal longi-

tudinal channels 11, illustratively located in the median plane M between the billet surfaces which are to be rolled. The organic resist materials act by preventing interpenetration of the metal laminate material through 5 the resist film and welding is prevented, and the film is continuous. It is not necessary to provide originally a thick resist layer as with the use of refractory powder resist where the resist residue must be several granules thick at the end of cold rolling; and hence a channel 11 10 may be  $\frac{1}{8}$  inch thick or less, even with a 12 inch ingot which is to be rolled to a final thickness of 0.016 inch, or an extension of 700 times.

It has been found preferable, with resists which are liquid during the early or breakdown stages of the hot 15 rolling, to have the channels 11 with edges of chisel-shape, as shown in FIGURE 1, with the upper and lower surfaces of each channel formed by parallel planes, and with the edges of each channel formed by convergently tapered surfaces which have an angle of 10 to 90 degrees 20 relative to one another. Practices with angles of 14 and 28 degrees show that there is little difference between them for the liquefied resists above. The tapered surfaces can be planes which merge by minor curvatures with the aforesaid parallel surfaces, and which are joined 25 by a curve of small radius: e.g., with channels  $\frac{1}{8}$  inch thick, the edge curvature can be around  $\frac{1}{64}$  inch in radius. During the initial rolling, the liquid resist coats the internal surfaces: and as the metal is forced together at the channels, the tapered edges provide smooth transitions 30 so that internal roughness does not develop.

Channels of other cross-sections can be employed in accordance with the invention. In FIGURE 2, the channels 11a are oblong, with rounded contours at the edges. In the initial hot-rolling, the upper and lower surfaces 35 of such channels move toward one another, and the resist maintains its coating upon the internal surfaces; ultimately providing a film of essentially uniform thickness.

In FIGURE 3, the channels at the end 12 of the ingot are shown as closed by peening and a welded seam 13, it being understood that this closure extends across and closes the entire end in the complete ingot. With the sealed end down, FIGURE 4, the resist material may be introduced as a slab, sheet, or powder, e.g., through a guide or hopper 14. When the resist makes contact with 40 the hot channel walls, FIGURE 4, as it moves downward, it melts thereagainst to provide a coating: when a strip  $\frac{1}{16}$  inch thick and 2 or 3 inches wide is thus fed, lateral movements during feeding and while within the channel assure the coating: like spreading occurs with 45 powder particles. This coating effect is assisted by foaming and bubbling of the resist, FIGURE 4; in practice, by the completion of the feeding, fumes are billowing out, displacing the air from the channel. If the ingot has been 50 previously heated, as stated above, the resist melts, discharges its air of porosity and its volatiles, if any, and the upper end 15 can now be peened and welded shut so that the resist material is totally enclosed against entry of gases from the atmosphere and against escape of any resist material. Alternatively, the billet can be quickly 55 brought to horizontal position, without sealing its open end, and pushed into the rolls. If the ingot is cold, the resist can be introduced, with tamping and vibration to assure a tight filling, and then peened and welded shut.

The loaded and closed billet B is then subjected to its 60 schedule of heating and rolling. With aluminum and its alloys, this is usually a heating 30, FIGURE 5, to 900 degrees F., with a succession of hot-rolling passes 31 to reduce the material to about four to eight times the desired final thickness. The hot-rolled strip is then annealed in step 32 at 900 degrees F. for 30 minutes, cooled, and subjected to a succession 33 of cold-rolling passes to bring it to final thickness as a strip S. More than one intermediate annealing can be employed, as set out above.

When the rolling can be conducted immediately upon 65 loading the billet channel with organic resist, as in Ex-

amples 1, 2 and 3 above, the billet may be brought to the desired condition and temperature for hot-working before the resist is introduced. For example, an aluminum alloy ingot B, FIGURE 6, can be heated to 900 to 1,000 degrees F., and a resist in liquid form can then be inserted into the channel at the end which is initially to be fed into the reduction rolls 16. This can be done by an injecting pump cylinder 17 having a nozzle 18 which enters a channel or discontinuity 19 of the billet B, and deposits a quantity of the resist within the channel at the leading end, as shown by the dotted lines 20, continuing the deposit until the nozzle is fully withdrawn. When the billet has several channels, it is preferred to charge all channels at the same time, so that air-exposure of heated resist is kept to a minimum time. The billet B is immediately introduced to the rolls 16 and a reduction made which closes the walls of the channels 19 upon the resist so that air access thereto is thereafter prevented, and the resist is spread and distributed between the internal wall surfaces, being pushed along the channel during the rolling and the excess squeezed out as the rolling pass is ended. Therewith, the resist provides a thin film which prevents welding of such internal surfaces. Silicone greases or oils having the polysiloxane structure of a chain of silicon and oxygen atoms, with the silicon atoms having hydrocarbon groups connected thereto, for example of the formula



(e.g., the commercial material sold under the trademark DC-710) can be so employed, with the pump delivering the resist at a room temperature of 70 degrees F., or a temperature of below 500 degrees F., e.g., 300 to 400 degrees F., at which there is essentially no degradation upon air contact during the time for injecting and the early rolling. The resist is immediately heated from the hot billet, upon injection, but then it is protected against major contact with oxidizing substances such as air. Minor degradation can occur between the surface of the mass and the air present in the channel, but in practice, this has not been found harmful when the rolling is started quickly. There appears to be a time function for the degradation, so that when the hot-rolling at temperatures above, say, 600 degrees F. is completed within five minutes, the silicone continues effective for the hot rolling, and during a subsequent cold rolling. When such a strip has been cold-rolled to final gauge, and is heated for 30 minutes or more for annealing, the silicone decomposes, with the production of negligible amounts of gas and silica per unit area of the laminate stock, and no notable bulging of the laminations away from one another.

This pre-heating of the billet to hot-rolling temperature, and the immediate hot-rolling, can be employed with the several resists and metals described above. It is applicable with other organic compound resists having the stated characteristics and even with resists which undergo polymerization at hot-rolling temperature, provided that the hot-rolling is completed before polymerization has progressed to a stage at which the anti-welding effect is not maintained during the course of the rolling schedule. For example, if the compound requires two minutes or more for the polymerization to a condition in which the product is no longer thermoplastic or extensible under rolling pressure, it can be used in a schedule of hot rolling and cooling to a temperature at which the progress of polymerization is slow; because it is feasible in practice to conduct the hot-rolling of selected billet sizes and the cooling within two minutes, with the resist then present in a form proper for cold rolling.

In practice, in making tubular bodies of 12 inches diameter or less, it is economical to form the original bil-

let with more than one channel 11, or 11a, as shown in FIGURES 1 and 2: but it will be understood that the invention can be employed with billets having a single channel and that, for some employments such as the making of heat exchange bodies, the internal channels may be connected within the billet body. Therewith the billets need not be original hollow ingots, but can be prepared by other procedures known in the art of making laminate stock, with care taken to assure the closure of each channel or group of channels against atmosphere penetration or the escape of resist material into places where it can interfere with the regular course of reduction of the billet. Thus the channels may be provided by casting molten metal about cores which are later removed, by casting molten metal about hollow tubes which become integrated with ingot metal, or by boring or piercing.

The strip S (FIGURE 7) has a number of longitudinal internal resist residues 35 equal to the number of channels 11 or 11a in the original billet; and these residues may be present in such thin layers that they are each represented by a single line in the drawing. These residues 35 separate the metal laminations 36, 37, with the laminations connected at the lateral edges of the resist residues by the longitudinal metal portions 38. When more than one channel and residue is present, the strip S can be called "multi-wide" because it can be parted into a number of "single-wide" strips by severance, as represented by the line 39, along upright surfaces which extend along the metal connections 38 between adjacent residues 35 so that each strip retains a part of such connection. The edges of the strip S may likewise be severed at surfaces represented by the line 40, so that each single-wide strip has edge connections of essentially the same lateral dimensions from the corresponding edges of the resist residue. 35 Decoration, such as the printing of pictures and words can be done, before or after severance into blanks, and the laminate stock can be embossed with ribs and grooves for stiffening the walls after opening: wherewith the resist residue continues to act to prevent internal sticking or welding. The strip S can likewise be severed transversely to provide container body blanks, which are opened or expanded as shown in FIGURE 8, wherewith the laminations 36, 37 provide the major portions of the tubular bodies T; and therewith the wall thicknesses of the bodies 40 are determined by the final rolled gauge of the strip, being illustratively half this gauge because the resist layer 35 can be of insignificant thickness. The parts of the integral connections 28 for the specific body T are present as externally projecting fins 41 which may be trimmed and conformed to the general body cross-section, FIGURE 9. 45 When the resist material is selected from the substances described in the examples, the residue is adherent to the internal walls of the body T, and is compatible with organic enamels and lacquers. Thus, after the fins 41 have 50 been conformed as shown in FIGURE 9, wherewith the reentrant angles 42 have been essentially removed at the interior, an enamel may be applied as by the conventionalized spray nozzle 45 during passage of the body along the same. The enamel can then be dried and baked. 55 Illustrative organic enamels or lacquers have "solid" components of oleo-resins, phenolic resins, epoxide resins, or vinyl resins along with pigments and fillers; and include resin solvents such as hydrocarbons, ketones and esters. Solvents which dissolve the resist residues merely form a 60 modified organic coating, assuming the resist resin residue and the added resin are compatible. When the solvents do not act upon the resist residues, and are eliminated during drying, a fluxing together of the resist residues and the enamel resins can occur during baking. 65 Organic resists which have been found effective for the procedure have the common chemical and physical attributes that they have a molecular weight above 500; exhibit thermoplasticity, i.e., being liquid, upon heating under non-oxidizing conditions in the range of 500 to 1,000 70

degrees F. so that they respond during the extension of the metal area and are deformed uniformly therewith; and do not change by degradation or polymerization during such heating and pressure in the absence of air so that such response is not exhibited. "Thermoplasticity" herein has the usual meaning of capability of being deformable without rupture or significant decomposition when heated above room temperature. It has been found that the materials can be tested as to behavior during rolling, by filling a tube, made of the metal which is to form the laminate stock, substantially full with the material, sealing the ends as by welding, and heating to the proposed operating temperature, e.g., 900 degrees F. for one hour. Upon cooling and opening the tube, the material is then examined as to appearance, solubility, infra-red analysis of the molecular structure, and physical condition at room and elevated temperatures. The useful materials, then, exhibit thermoplasticity and cohesion under pressure, and upon infra-red analysis exhibit a pattern or graph essentially the same as the untested material.

The properties of the useful organic resist materials include the ability to endure the temperatures of heating, with exclusion of oxygen, e.g., air, without loss of anti-welding properties, so that they continue effective for that purpose through the course of reduction, illustratively by a schedule of hot and cold rolling preferably with a maintained adhesion to the metal surface which is greater than the internal cohesion within the resist layer, and the ability to accept and establish adhesion to organic enamels later applied thereto. When the produced strip material is to be in contact with foodstuffs, e.g., when the tubular body T of FIGURE 6 is to be part of a food container, the resist material should not comprise a toxic component or have a toxic or flavor-change effect. The resist material should extend regularly and in proportion to the extension of length and reduction of thickness of the billet metal, so that smooth internal surfaces are produced: that is, it should be extensible. These properties are presented by the materials of the examples; the internal surfaces of Example 9 with aluminum metal and silicone resist exhibited excellent dry adhesion for organic enamels, but when subjected to the standard spinach-oxygen test and stored for four days, there was some loss of enamel adhesion.

The continuity of the residual resist films on the internal wall surfaces on laminate stock prepared from an aluminum alloy (commercially known as 6061) was tested by treating a standard area with air-free citrate buffer solution of pH 3.5 at 100 degrees F. Comparable bare aluminum alloy surfaces are thereby attacked, and hydrogen gas is evolved at a rate of 0.100 to 0.120 milliliter (measured at standard temperature and pressure) per square inch per day. With polyethylene resist as in Example 4, Z-6018 silicone resist as in Example 9, and Epon 1007 resist as in Example 1, the hydrogen evolution was 0.052 to 0.059 milliliter per square inch per day, showing that the extremely thin residual material was present as a protective agent.

In general, the satisfactory resist or anti-welding materials may be defined chemically as organic compounds (the term as usual including the silicone compounds having hydrocarbon groups in the molecular structure) which are waxy, rubbery, or resinous in behavior at room or slightly elevated temperatures, which endure exposure to temperatures around 900 degrees F. in the absence of oxygen, and which have a molecular weight above 500.

Among the useful organic compounds so defined are:

(a) Resinous polymers of  $-(CH_2\cdot CR)_n-$  structure, where R can be hydrogen, alkyl hydrocarbon groups of 1 to 4 carbon atoms, phenyl, alkyl-substituted phenyl, and polyalkyl-substituted phenyl, and n denotes the presence of a plurality of such units in chain (inclusive of the resins known as polyethylene, polypropylene, polystyrene, polymethylstyrene, polyvinyl-toluene, polybutene, copoly-

mers of polybutene with polyethylene and/or polypropylene):

(b) Metal soaps of the structure  $(R^2\cdot CH_2\cdot CO_2)_p\cdot R^3$ , where  $R^2$  is an aliphatic or olefinic hydrocarbon group of 5 to 16 carbon atoms,  $R^3$  is a metal ion, and p denotes a number of acid groups no greater than the replacement valency of the metal whose ion is being used (inclusive of sodium and other monovalent metals, calcium and other bivalent metals, aluminum and iron and other trivalent metals, and of the stearates and oleates):

(c) Essentially linear condensation polymers of the structure  $== (R^4\cdot CO\cdot R^5\cdot CO)_q ==$ ; where  $R^4$  represents a normal hydrocarbon group of 2 to 10 carbon atoms, isopropylidene-bis-(para, para prime-phenoxy),

$== (normal C_5H_{10}\cdot NH) ==, -O\cdot R^6\cdot O-$

and  $-NH\cdot R^6\cdot NH-$ ;  $R^6$  represents a normal alkyl hydrocarbon group of 2 to 10 carbon atoms, meta-phenylene, para-phenylene,

$== (normal C_5H_{10}\cdot NH) ==$

and isopropylidene-bis-para, para prime-phenoxy;  $R^6$  represents a normal alkyl group of 2 to 10 carbon atoms; and q denotes the presence of multiple units in chain (inclusive of polycarbonates, polyamides such as the linear carboxylic acid:amine condensations including dibasic acid:diamine polymers and caprolactam polymers, and polyesters, e.g., of terephthalic, isophthalic, adipic and sebatic acids with ethylene glycol, propylene glycol and homologous glycols):

(d) Thermoplastic resins having multiple phenyl nuclei in chain, to wit: phenol-aldehyde or phenolic resins (inclusive of the novolacs such as para-phenyl-phenol:formaldehyde condensate resin), and epoxy resins with multiple phenyl nuclei (inclusive of the bis-phenol epichlorohydrin condensates):

(e) Polyorganosiloxanes or so-called silicones having alternate silicon and oxygen atoms in chain with the free valencies of the silicon atoms joined to hydrogen or hydrocarbon groups directly or through oxygen (inclusive of the linear silicone polymers and of the compounds with ring structure or cyclic tetramer units as in Example 6 above, and of thermoplastic compounds having molecular cross-linkages through oxygen atoms between silicon atoms of two or more chains):

(f) Polyterpene resins.

The heating and presence in enclosed channels, during the process, prevents entry of oxygen from the air. General decomposition reactions of organic compounds can cause gaseous products, and the pressure thereof causes a shifting of the equilibrium point so that the reaction ceases when the sealing prevents escape. In practice, it has been found that the decomposition or depolymerizations occurring, which do not yield gaseous products, are apparently without destructive effect upon the selected resist materials, noting the results of practice and infra red examination as stated above. Polymerization of originally high molecular weight materials also is not deleterious, provided that an infusible, highly brittle product does not result so that the antiwelding capability is lost during completion of the reduction operations.

The procedure comprises the exclusion of oxygen while the billet is at elevated temperature. This is preferably done by sealing the channel against entry of air: but under the invention the exclusion may be effected in other ways.

For example, after first heatings and rollings, the ends may be clipped and the rolling continued. It has been found that with a silicone resist material in an aluminum billet, the ends could be peened without welding, so that part of the resist was extruded in the first rolling pass: the laminate stock after rolling to gauge was found to open easily and had a good internal appearance.

Another practice of the use of high molecular weight organic resists is that of conforming the billet to the resist or anti-welding material before heating to the temperature required for hot-rolling the billet metal. Thus, a billet

having its channel partly filled with the resist may be initially rolled at a temperature below that at which the resist is degraded upon air contact; whereby to distribute the resist, expel air, and conform the billet to the resist without air-filled pockets or spaces. Such a temperature can be a cold rolling condition for the metal, and one at which the resist extends easily under roll pressure effects upon and in the billet and is for example a stable fluid. The degree of reduction can be small during this initial conformance rolling, e.g., with a billet 8 to 14 inches thick and the longitudinal channel  $\frac{1}{4}$  inch thick, the over-all reduction of thickness may be less than 5 percent, and essentially no cracking develops. No internal pressure need develop, as the end or ends may be left open for escape of air and excess resist.

A billet having one or more channels, closed at the lower end as in FIGURE 4, receives the resist material at room temperature or at between room temperature and about 500 degrees F., at which the resist is liquefied but not damaged by heating in contact with air. A suitable temperature for the described organic compound resists is 300 to 400 degrees F. It is difficult and often expensive to prepare billets with a channel less than around  $\frac{1}{8}$  to  $\frac{1}{4}$  inch in thickness; noting that a greater original thickness of resist is not required to maintain the anti-welding action, since upon reduction of such channel to microscopic thinness, e.g., one ten-thousandth of an inch or less, the welding is still prevented. Hence, the channel cavity can be filled part full of liquid resist or partly filled with a strip of resist material much thinner than the channel. The billet is then rolled at a temperature, room or above, at which the resist is not damaged by air contact, by light passes until the resist is spread evenly over the channel surfaces, and therewith the billet has its channel thickness reduced to conform to the resist present and thus the residual channel space is full, with expulsion of air and some of the resist material. The billet is then heated to the temperature at which the hot-rolling of the metal is to be started, e.g., 900 to 1,000 degrees F. for aluminum and its alloys, and the schedule of hot-rolling performed.

In practice, an advantage of the very thin resist residues is that intermediate annealing or reheating can be conducted during the course of the hot-rolling without causing bulging or expansion, which may occur if a large thickness of resist having a gaseous product or an appreciable vapor tension at the heating temperature, is present. The billet and the resist afford mutual protection to each other: the billet encloses and protects the resist from decomposition or vapor formation, and the resist prevents oxidation of surfaces of the billet channel or channels. The final laminate stock has bright and clean internal surfaces. With these practices of lightly rolling the billet to reduce the channel dimension before heating to rolling temperature, it is preferred to have the channels 49 of rounded-end section, as in FIGURE 1, or of elliptical cross-section, as shown in FIGURE 2, because therewith, the residual cavity after rolling has a more uniform thickness without excess thickness at the lateral edges of the reduced channels, such as may be present after a light schedule of early rolling with channels of rectangular section.

When a silicone grease or oil (such as that commercially known by the tradename DC-710) is used, it can be employed at 70 degrees F., and the conformance rolling done at this temperature. With polyethylene, a temperature of 300 degrees F. can be employed. Suitable temperatures for other compositions are indicated in the examples.

In forms of practice in which the resist is brought into a billet already heated to hot-rolling temperature or in which the billet is heated to such temperature with the resist therein, and then forthwith subjected to hot-rolling, the developing of gas by degradation of a part of the resist is frequently of assistance in providing a plenum effect, so that the entry of air is prevented. Such gas

evolution is greatest at the start of a rolling schedule: and drops as the metal cools during and between rolling passes. In addition, the extension of the length of the channel and its reduction of thickness hinder and prevent the travel of any evolved gas along the channel.

5 The procedure is effective with metals which can be rolled at temperatures of 1,100 degrees F. or below: inclusive of aluminum, zinc, copper, magnesium and other non-ferrous metals and their alloys: and is particularly 10 of value with such materials which require hot-rolling or heat-treating temperatures of 500 to 1,100 degrees F.

In accordance with this procedure, the resist is preferably a liquid during initial rolling passes so that it conforms to the channel; and exhibits increased viscosity during later rolling passes at temperatures below 500 degrees 15 F. and down to room temperature.

The procedure includes the employment of original resist channels of such original thickness that insignificant thicknesses of resist residues are present in the final 20 step, e.g., below 0.001 or 0.0005 of an inch. This is particularly valuable when the adhesion of the resist residue to the metal is greater than the internal cohesion of the resist so that, upon opening or expansion, the inner surfaces of both metal laminations have films of the resist residue thereon, with the separation usually making 25 the films of essentially the same and like thickness throughout. For this, it is preferred to execute the rolling with reversal of the billet at successive passes: that is, the trailing end at one pass is made the entering end 30 at the next pass, so that any effect of longitudinal movement of the resist, independently of the metal extension and with an effect of increasing the relative resist thickness at the trailing end compared to the entering end, is compensated by the reverse rolling. Therewith, the fluidity 35 of the resist expelled at the trailing end of the billet is not as destructive, e.g., by abrasion, as a resist of solid refractory particles would be when the trailing end is immediately fed to the rolls for the second or reverse pass.

It has been brought out above that the necessary residual thickness of resist material, in the final strip, can be very small, that correspondingly a very thin channel can be effective in a thick ingot, that technical considerations restrict the minimum channel thicknesses which can be provided in ingots, and that in fact the quantity of 45 original resist material can be less than that for filling the channel, as shown by the expulsion of a large part of the originally introduced resist at the end of the first and subsequent hot-rolling passes. The action during the first hot pass is, on the one hand, to conform the ingot to the resist so that air is expelled and its re-entry prevented; and on the other hand to spread the resist so that it fills the reduced channel with coverage at all surfaces thereof. In practice, where both ends of a channel were closed by welding, the movement of liquid resist along 50 the channel incidental to the rolling causes such a high pressure to develop that the closure at the trailing end of the ingot bursts open and excess resist is expelled. Comparably, with FIGURE 6, for example, where the trailing end can be open, a like expulsion occurs.

60 In some cases, where the hot rolling temperature makes the resist a thin liquid and there is rapid rolling of a billet which is open at the trailing end, the resist may be caused to travel along the channel at high velocity and without the amount of lateral spreading required to coat the entire internal surfaces. This is revealed during the 65 hot rolling by proper coating of the inner surfaces for the first half of the billet, for example, and by the lack of full coating at the channel edges for the second half of the billet; so that local pressure welds occur at the channel edges, with decrease of the width of the resist residue at such pressure-welded regions in the final strip whereby parts of the strip must be discarded if accuracy of width is demanded.

70 It has been found that in such cases coating of the internal surfaces can be improved by a roughening of the 75

internal surfaces. Such roughening need not be and preferably is not of major extent. For example, after an ingot has been cast with one or more internal channels, of say 0.120 inch thickness, and these are broached or burnished, a roughening not perceptible by touch will produce a retardation of the longitudinal flow of the liquid resist, during rolling, with development of a back pressure effect which causes lateral spreading and coating. Such a roughening can be produced by etching: for example, with aluminum and aluminum alloys, a treatment with hot caustic alkali solution for a few minutes, following by rinsing produces a microscopically rough surface, of the order of 10 to 50 micro inches between hills and valleys. This etching and rinsing is preferably done before the ends are closed. Upon introduction of the resist either with sealing of the ends as in FIGURES 3 and 4 or without such sealing as in FIGURE 6, the roughened surfaces act to detain the resist at the metal: resist boundaries of the channels during the courses of the rolling passes. Upon hot rolling, the longitudinal extension of the billet to strip form gives internal surfaces, after opening, which have a somewhat matte appearance but without significant depths of the surface irregularities.

In cases where a great reduction of thickness is scheduled, particularly in cold rolling passes, and the residual film of resist may become too thin or discontinuity may develop therein, the invention permits the replenishment of resist. For example, the leading end of the strip can be opened, more liquid resist of the same or a different type introduced, and the rolling continued, wherewith the added resist mass is caused to travel along the channel during the rolling and re-establish a desired film thickness for successive rolling passes. It is notable that this cannot be accomplished with resists which are granular, refractory solids, and do not have the flow properties for such replenishment.

The invention is not limited to the illustrative forms, and may be practiced in many ways within the scope of the appended claims.

What is claimed is:

1. The method of producing a laminate metal stock which comprises preparing a billet of a metal selected from the group consisting of aluminum, zinc, copper, magnesium and their alloys, and said metal requiring a hot-rolling temperature of 500 to 1100 degrees F., said billet having an internal cavity, introducing into the cavity an organic compound having a molecular weight above 500 and which at the temperature for hot rolling of the metal is a liquid and is extensible at cold rolling temperatures for the metal and heating the said organic compound to lower the viscosity of the same to a condition for easy spreading, reducing the billet at a temperature between 500 and 1,100 degrees F. for closing the cavity surfaces upon the said organic compound and thereby expelling gases from the cavity, and spreading the said organic compound and therewith coating the cavity surfaces with the said organic compound, and continuing the reduction with air excluded from the cavity in the metal undergoing reduction, said heating and reduction including at least one step of bringing the billet to a temperature of 600 to 1,100 degrees F. with the said organic compound contacting the billet cavity walls at such temperature.

2. The method as in claim 1, in which the said organic compound is a resin having units of the structure



where R is selected from the class consisting of hydrogen, alkyl groups of 1 to 4 carbon atoms, phenyl, alkyl substituted phenyl and polyalkyl substituted phenyl, and n denotes the presence of a plurality of the units in chain.

3. The method as in claim 2, in which the said organic compound is polyethylene.

4. The method as in claim 1, in which said organic compound is a metal soap of the structure



5 where R<sup>2</sup> is selected from the class consisting of aliphatic and olefinic hydrocarbon groups of 10 to 16 carbon atoms, R<sup>3</sup> is a metal ion, and p is a number not greater than the replacement valency of the metal whose ion is selected.

5. The method as in claim 4, in which the organic compound is iron stearate.

10 6. The method as in claim 1, in which the said organic compound is an essentially linear condensation polymer having units of the structure



15 where R<sup>4</sup> is selected from the class consisting of normal alkyl hydrocarbon groups of 2 to 10 carbon atoms, isopropylidene-bis-(para,para'-phenoxy),



—O—R<sup>6</sup>—O—, —NH·R<sup>6</sup>·NH—; R<sup>5</sup> is selected from the class consisting of normal alkyl groups of 2 to 10 carbon atoms, meta-phenylene, paraphenylene,



20 and isopropylidene-bis-(para, para'-phenoxy); where R<sup>6</sup> is a normal alkyl group of 2 to 10 carbon atoms; and q denotes the presence of multiple units in chain.

7. The method as in claim 6, in which the said organic compound is a polycarbonate resin.

25 8. The method as in claim 1, in which the said organic compound is a condensation polymer selected from the class consisting of thermoplastic resins derived from the reaction of phenols with aldehydes, and epoxy resins with multiple phenolic nuclei.

9. The method as in claim 8, in which the said organic compound is a bis-phenol epoxy resin.

10. The method as in claim 1, in which the said organic compound is a polyorganosiloxane.

30 11. The method as in claim 10, in which the said organic compound is a polysiloxane having units of the structure



45 50 where R<sup>7</sup> is phenyl, R<sup>8</sup> is an isopropyl group, and t denotes the presence of multiple units in chain.

12. The method as in claim 1, in which the metal is aluminum and the hot-rolling is conducted from a temperature of 700 to 1,100 degrees F.

13. The method as in claim 1, in which the metal is a copper base alloy, and the said organic compound is introduced while the billet is at a temperature of about 950 degrees F. and the billet is hot-reduced from such temperature.

60 14. The method as in claim 1, in which the hot-reduction is at successively lower temperatures, and a final cold-reduction is employed to attain the desired final dimensions.

15. The method of producing a laminate metal stock which comprises preparing a billet of a metal selected from the group consisting of aluminum, zinc, copper, magnesium and their alloys, and said metal requiring a hot-rolling temperature of 500 to 1,100 degrees F., said billet having a longitudinal internal channel with an open end, introducing through said end and into the channel an organic compound which at a temperature for hot-rolling of the metal is a liquid and subject to decomposition in air and is extensible at cold-rolling temperatures for the metal, thereafter rolling the billet while at a temperature of 500 to 1,100 degrees F. for closing the channel surfaces

upon the said organic compound and thereby expelling gases and a quantity of said organic compound from the channel, and continuing the rolling while the metal is at a hot-rolling temperature and with air excluded from contact with the organic compound by the metal undergoing reduction.

16. The method as in claim 15, in which the surfaces of the internal channel are first smoothed and thereafter etched before the introduction of the organic compound.

17. The method as in claim 15, in which the said organic compound is introduced into the channel while the billet is below the temperature of decomposition of said organic compound while in contact with the air, and in which the said open end is closed before the billet is heated to hot-rolling temperature.

18. The method as in claim 17, in which the said organic compound is a liquid at a temperature below 500 degrees F., and the billet is warmed to a temperature below 500 degrees F. for liquefaction of the said organic compound before the same is introduced.

19. The method as in claim 17, in which the said open end is closed before the billet is rolled for reducing the channel surfaces upon the said organic compound.

20. The method as in claim 15, in which the billet is heated to hot-rolling temperature before the said organic compound is introduced, and is immediately subjected to rolling for closing the channel surfaces upon the said organic compound and expelling air.

21. The method as in claim 15, in which the billet is subjected to a succession of hot-rolling passes and the direction of billet entry between the rolls is reversed for successive passes.

22. The method of making laminate strip stock, which comprises introducing into a longitudinal internal channel of a billet of metal which requires a temperature of 600 to 1,100 degrees F. for hot-rolling an organic compound which at the hot-rolling temperature for the metal is subject to decomposition in air and is a liquid at a temperature above room temperature and below 500 degrees F. and is extensible at cold-rolling temperatures for the metal, and hot-rolling the billet by successive passes from a temperature of 900 to 1,100 degrees F. and thereafter cold-rolling the hot-rolled strip.

23. The method as in claim 22, in which the billet is heated to hot-rolling temperature before the introduction of the organic compound, is immediately subjected to the hot-rolling, and reduced to a temperature below 500 degrees F. within five minutes after the introduction of the organic compound.

24. The method as in claim 23, in which the channel is open at one end, and the organic compound is introduced for a limited zone adjacent said open end, and the billet is immediately brought to hot-rolling with the open end presented to the rolls.

25. The method of producing a hollow metal body having an internal coating of a selected organic enamel composition, which comprises introducing into an internal cavity of a billet of metal selected from the group consisting of aluminum, zinc, copper, magnesium and their alloys, and said metal requiring a hot-rolling temperature of 500 to 1,100 degrees F., an organic compound which is a liquid and subject to decomposition in air at a temperature for hot-rolling of the metal and is extensible at cold-rolling temperatures for the metal and is compatible

with the selected enamel, heating the said organic compound to melt the same within the cavity, hot-reducing the billet at a temperature of 600 to 1,100 degrees F. for bringing the cavity surfaces into conformity with the liquefied organic compound and for producing the desired shape with the surfaces of the cavity separated by the organic compound and with the organic compound protected from the air by the metal of the billet, then cold rolling the hot-reduced product thereafter moving cavity surfaces apart to provide the internal hollow of the body, and applying the organic enamel composition to the resist-coated internal surfaces.

15 26. The method of producing a hollow tubular metal body, which comprises introducing into a longitudinal internal channel of a billet of metal which requires a temperature of 600 to 1,100 degrees F. for hot-rolling a thermoplastic organic compound which at the hot-rolling temperature for the metal is a liquid and subject to decomposition in air and is extensible at cold-rolling temperatures for the metal, heating the said organic compound to melt the same within the channel, hot-rolling the billet at a temperature of 600 to 1,100 degrees F. for bringing the channel surfaces into conformity with the liquefied organic compound and expelling a part of the organic compound from the channel and effecting contact of the organic compound with the surfaces of the channel throughout its length, continuing the hot-rolling and thereupon after cooling effecting cold-rolling for producing a laminate strip having laminations separated by the residue of the organic composition and connected at their edges by integral metal from the billet, and moving the laminations apart for forming the tubular body.

20 27. An article of manufacture comprising a cold and hot-rolling laminated metal strip having at least one longitudinal internal channel containing a continuous microscopic film of less than 0.001 of an inch thick; said film consisting of an organic resist compound capable of decomposing in air at temperatures above 600° F. and having been subjected to the hot-rolling temperatures of about 900-1,100° F. in the absence of air; and laminations being integrally connected by metal along the longitudinal edges.

28. The article of claim 27 further characterized as a hollow metal body formed from the laminated metal strip; said hollow metal body having integral walls, the inner surfaces of which contain an enamel-coating composition which is compatible with said film of the organic-resist compound.

#### References Cited by the Examiner

##### UNITED STATES PATENTS

- |           |      |                          |
|-----------|------|--------------------------|
| 2,986,810 | 6/61 | Brick.                   |
| 2,990,608 | 7/61 | Manning ----- 29-470.9 X |
| 3,029,155 | 4/62 | Maier ----- 29-423 X     |

##### FOREIGN PATENTS

- |         |      |                |
|---------|------|----------------|
| 227,369 | 8/59 | Australia.     |
| 774,008 | 5/57 | Great Britain. |
| 814,979 | 6/59 | Great Britain. |

WHITMORE A. WILTZ, Primary Examiner.

HYLAND BIZOT, Examiner.